

## UNITED STATES PATENT OFFICE.

LOUIS A. WALKER, OF FRANKLIN, PENNSYLVANIA, ASSIGNOR TO THE FRANKLIN RAILWAY OIL COMPANY, OF FRANKLIN, PENNSYLVANIA, A CORPORATION OF DELAWARE.

## SOLID LUBRICATING COMPOUND.

No Drawing.

Application filed November 21, 1925. Serial No. 70,688.

This invention relates to a solid lubricating compound of the class usually termed driving journal compound, its principal use being in the lubrication of the driving journals of railway locomotives. My improved lubricant is also suitable for the lubrication of other high speed, heavy bearings as well as for the bearings of the driving-rods of locomotives. A lubricant used for the last-named purpose is usually termed a rod-cup grease.

In compounding my improved lubricant in accordance with this invention, I employ the following ingredients in substantially the proportions specified, namely:

|                              | Per cent. |
|------------------------------|-----------|
| Paraffin-base cylinder stock | 49        |
| Stearic acid                 | 39.25     |
| Alkali (e. g. caustic soda)  | 7         |
| Water                        | 4.75      |

These ingredients are compounded and mingled in an open-top, steam-jacketed kettle having a capacity of not less than four times the bulk of the original batch of ingredients so that the mass may not overflow the kettle during the interval of reaction due to saponification.

Said ingredients are charged into the kettle as, and in the order named and in the course of such charging temperatures are maintained as follows:

The stearic acid is first placed in the kettle and a suitable degree of steam heat is applied to melt the same, but the degree of heat at this stage should not exceed 200° F.

The cylinder stock is next added, at which interval the degree of heat remains the same: Agitation is employed throughout this interval.

The alkali in solution with the amount of water previously given is lastly added, agitation being continued throughout this interval, and thereafter to the end of the compounding process.

As the alkali solution is added a vigorous reaction of saponification is set up and this causes an autogenous generation of heat whereby the temperature of the mass is raised to approximately 230° F.

Throughout this interval of reaction water is expelled from the mass in dense clouds of

steam. Reaction is further indicated and attended by an intense foaming and a very material increase in the bulk of the mass. The steam heat applied during this interval must be carefully regulated in order that the batch may not overflow the kettle. 55

A completion of the reaction of saponification is indicated by a cessation of increase in the bulk of the mass, and at the point of such cessation pressure of steam in the jacket of the kettle is raised to the final pressure of approximately 110 pounds which is equivalent to a heat of 345° F., and this degree of heat is utilized for the purpose of cooking 60 the compound.

Agitation is continued throughout the cooking process, which is continued until the batch indicates a tendency to draw away from the sides of the kettle, to ball up on 70 the agitator and to be moved en-massé thereby, thus indicating a completion of the process of compounding and a proper and suitable condition of the compound.

The compound produced as above stated 75 is what is known as a fibrous lubricant, it has a density approximately equal to that of a laundry soap and gives the following analysis:

|                 | Per cent. |
|-----------------|-----------|
| Cylinder stock  | 52.5      |
| Sodium stearate | 46.0      |
| Free alkali     | 00.5      |
| Water           | 1.0       |

In specifying the proportions of ingredients originally entering into my compound, due consideration is had for the fact that cylinder stock may vary somewhat as to its fire test, and the proportions specified contemplate a stock having a fire test of 85 600° F. For further characteristics of cylinder stock see the publication entitled American Petroleum Industry Vol. 2, page 362, by Bacon and Hamor.

Any fatty acid that is a close chemical 95 equivalent to stearic acid may be employed in place thereof.

My improved lubricating compound has, upon account of the greater proportion of mineral oil,—cylinder stock—which it contains, superior lubricating efficiency. Said 100 superior efficiency is largely due to the fact

that this compound deposits upon the surfaces to be lubricated, a better film of lubricant than has heretofore been possible to attain in the class of service in which the compound is most largely used.

Furthermore, I have definitely ascertained that when my improved compound is used in the bearings of locomotive driving journals that are located adjacent the fire-box and ash pan of the boiler, this lubricant is not impaired by the action of the excessive heat at these points, hence, in this further respect it is an improvement over previous compounds; said fibrous structure having been produced in the process of manufacture by both the reaction of saponification and agitation.

I claim the following:

1. A solid lubricant consisting of, a paraffin base cylinder stock, approximately 52%, sodium stearate approximately 46.5%, free alkali 0.5% and water 1%.

2. A solid lubricant having a fibrous structure and consisting of a paraffin base cylinder stock 52%, a higher fatty acid soap 46.5%, free alkali 0.5% and water 1%.

3. A solid lubricant, compounded by means of the agencies of heat, saponification and agitation from paraffin base cylinder stock 49%, stearic acid 39.25%, caustic

soda 7%, water 4.75%, the resulting compound having an analysis as follows,—

|                              | Per cent. |
|------------------------------|-----------|
| Paraffin base cylinder stock | 52        |
| Sodium stearate              | 46.5      |
| Free alkali                  | 0.5       |
| Water                        | 1         |

4. A solid lubricant, compounded by means of the agencies of both externally applied and autogenous heat, agitation and saponification from the following ingredients,—

|                              | Per cent. |
|------------------------------|-----------|
| Paraffin base cylinder stock | 49        |
| Stearic acid                 | 39.25     |
| Caustic soda                 | 7         |
| Water                        | 4.75      |

the resulting compound having a fibrous structure and the following analysis,—

|                        | Per cent. |
|------------------------|-----------|
| Mineral oil            | 52        |
| Higher fatty acid soap | 46.5      |
| Free alkali            | 0.5       |
| Water                  | 1         |

In testimony whereof I affix my signature.

LOUIS A. WALKER.